

## UNITED STATES PATENT OFFICE.

HERBERT FROOD, OF CHAPEL-EN-LE-FRITH, ENGLAND, ASSIGNOR TO FERODO LIMITED,  
OF CHAPEL-EN-LE-FRITH, ENGLAND.

## MATERIAL FOR FRICTIONAL AND WEARING PURPOSES.

No Drawing.

Application filed March 21, 1923. Serial No. 626,641.

*To all whom it may concern:*

Be it known that I, HERBERT FROOD, a subject of the King of Great Britain and Ireland, and a resident of Chapel-en-le-Frith, 5 in the county of Derby, England, have invented certain new and useful Materials for Frictional and Wearing Purposes, of which the following is a specification.

This invention relates to a process for 10 manufacturing a fabric for friction surfaces and wearing purposes.

Usually frictional and wearing fabrics of the kind referred to are saturated with the cementitious substance by immersion there- 15 in under atmospheric or elevated pressure or in vacuo. Owing, in some cases, to the nature or character of the cementitious sub- stance or binder and, in other cases, to some prior treatment of the fabric, it frequently 20 happens that the cementitious substance does not readily penetrate the fabric or the fibres, and the object of this invention is to provide an improved method and means of impreg- nation which will overcome such disadvan- 25 tage.

According to this invention, frictional and wearing fabrics of the kind referred to are 30 coated and bonded by the cementitious sub- stance or binder being "frictioned" into the fabric.

The binder may be "frictioned" into the fabric in any suitable way. I may employ 35 any of the known methods and means used for "frictioning" rubber and waterproofing compounds into fabrics for other uses. Con- 40 veniently, I may pass the fabric one or more times between rollers rotating at different speeds and apply the binder to that surface between which and the corresponding roller 45 relative movement or slip takes place. The rollers may exert any desired pressure on the fabric to force the binder thereinto and consolidate same, and the "frictioning" may be effected under applied heat (in which case 50 the rollers may conveniently be hollow and be heated internally by steam or otherwise suitably) or under the heat due to "friction- 55 ing" only. After applying the binder, the fabric is suitably treated to finish off and 60 harden the binder according to the nature thereof.

I may employ any suitable binder. For example, I may employ an enamel or the like of the kind described in specification of British Patent No. 4627 of 1909, or a binder 55 of the kind described in specification of British Patent No. 164772, or one of the known phenol-aldehyde condensation products. Alternatively, I may employ as a binder a mixture of dammar gum (20%), 60 rubber (10%), linseed or tung oil (20%), and suitable solvents, such as mineral naphtha, benzol and the like (50%) with or without animal glue or casein. Or I may employ a mixture of glue or casein and rubber, or 65 I may use chloro-naphthalene substitution products or sodium or potassium or other silicates or mixtures thereof.

When the finished fabric is to be coloured, I may dye the fabric in the piece before im- 70 pregnation, or the yarn before weaving, or the fibres in the mass, and employ a transparent binder or similarly colour or dye the binder. Alternatively, the colouring of the finished fabric may be effected solely by the 75 employment of a suitably coloured or dyed binder.

In some cases, the finished fabric may be provided with a metallic or other suitable base or foundation to which it may be se- 80 cured by riveting, cementing, stitching or otherwise appropriately. When composed of unwoven fibres or fibrous material, the fabric may have incorporated in it wires, wire netting or gauze, expanded metal or 85 other suitable reinforcement, and when composed of woven fibres I may provide the yarn with wire or other reinforcing centres or cores.

What I claim as my invention and desire 90 to secure by Letters Patent is:—

The process of manufacturing a friction fabric which consists in forcing a composi- 95 tion consisting of substantially two parts of dammar gum, substantially one part of rub- ber, substantially two parts of a drying oil, and substantially five parts of a solvent into a fabric by frictioning the composition into said fabric.

In witness whereof I have hereunto set 100 my hand.

HERBERT FROOD.